



US011453051B2

(12) **United States Patent**  
**Jablonski et al.**

(10) **Patent No.:** US 11,453,051 B2  
(45) **Date of Patent:** Sep. 27, 2022

(54) **CREEP RESISTANT NI-BASED SUPERALLOY CASTING AND METHOD OF MANUFACTURE FOR ADVANCED HIGH-TEMPERATURE APPLICATIONS**

(71) Applicant: **United States Department of Energy**, Washington, DC (US)

(72) Inventors: **Paul D. Jablonski**, Salem, OR (US); **Jeffrey Hawk**, Corvallis, OR (US); **Martin Detrois**, Salem, OR (US)

(73) Assignee: **United States Department of Energy**, Washington, DC (US)

(\*) Notice: Subject to any disclaimer, the term of this patent is extended or adjusted under 35 U.S.C. 154(b) by 0 days.

(21) Appl. No.: **17/184,542**

(22) Filed: **Feb. 24, 2021**

(65) **Prior Publication Data**

US 2022/0266332 A1 Aug. 25, 2022

(51) **Int. Cl.**

**B22D 25/06** (2006.01)  
**B22D 21/02** (2006.01)  
**B22D 18/06** (2006.01)  
**C22F 1/10** (2006.01)  
**F27B 14/06** (2006.01)  
**F27B 14/10** (2006.01)  
**C22C 19/05** (2006.01)

(52) **U.S. Cl.**

CPC ..... **B22D 25/06** (2013.01); **B22D 18/06** (2013.01); **B22D 21/025** (2013.01); **C22C 19/05** (2013.01); **C22F 1/10** (2013.01); **F27B 14/061** (2013.01); **F27B 14/10** (2013.01); **C22C 2202/00** (2013.01); **F27B 2014/066** (2013.01)

(58) **Field of Classification Search**

CPC ..... B22D 18/06; B22D 21/02; B22D 25/06; C22C 19/05; C22F 1/10  
USPC ..... 164/47, 61, 48, 492, 493, 495  
See application file for complete search history.

(56) **References Cited**

**U.S. PATENT DOCUMENTS**

|                   |        |                     |            |
|-------------------|--------|---------------------|------------|
| 5,443,111 A *     | 8/1995 | Colvin et al. ....  | B22C 9/061 |
|                   |        |                     | 164/254    |
| 6,561,258 B1 *    | 5/2003 | Kumpula ....        | C21D 8/005 |
|                   |        |                     | 148/335    |
| 2012/0110813 A1 * | 5/2012 | Bullied et al. .... | B22D 17/20 |
|                   |        |                     | 29/423     |
| 2014/0083645 A1 * | 3/2014 | Waniuk et al. ....  | B22D 35/04 |
|                   |        |                     | 164/493    |

\* cited by examiner

*Primary Examiner* — Kevin P Kerns

(74) *Attorney, Agent, or Firm* — Aaron R. Keith; Timothy L. Harney; Michael J. Dobbs

(57) **ABSTRACT**

One or more embodiments relates to a method of casting a creep-resistant Ni-based superalloy and a homogenization heat treatment for the alloy. The method includes forming a feed stock having Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B). The method further includes fabricating the creep-resistant Ni-based superalloy in a predetermined shape using the feed stock and at least one process such as vacuum induction melting (VIM), electroslag remelting (ESR) and/or vacuum arc remelting (VAR).

**19 Claims, 18 Drawing Sheets**





Prior Art  
FIGURE 1



FIGURE 2



FIGURE 3



FIGURE 4



(Prior Art)

FIGURE 5



(Prior Art)

FIGURE 6



(Prior Art)

FIGURE 7



FIGURE 8



FIGURE 9



FIGURE 10



FIGURE 11



FIGURE 12



FIGURE 13



(Prior Art)

FIGURE 14

Conv. Cast - Equiaxed



(Prior Art)

FIGURE 15



FIGURE 16



FIGURE 17



FIGURE 18

## 1

**CREEP RESISTANT NI-BASED  
SUPERALLOY CASTING AND METHOD OF  
MANUFACTURE FOR ADVANCED  
HIGH-TEMPERATURE APPLICATIONS**

**STATEMENT OF GOVERNMENT SUPPORT**

The United States Government has rights in this invention pursuant to the employer-employee relationship of the Government to the inventors as U.S. Department of Energy employees and site-support contractors at the National Energy Technology Laboratory.

**FIELD OF THE INVENTION**

Embodiments relate to a Ni-based superalloy casting and method of manufacture such a superalloy casting for advanced high temperature applications. More specifically embodiments relate to creep resistant NiCrCoAlTi (Ni-based) superalloy casting and method of manufacture the same for advanced super critical carbon dioxide (sCO<sub>2</sub>) power cycles.

**BACKGROUND**

Coal-fired boilers and steam/CO<sub>2</sub> turbines have operating temperatures greater than 760° C. over the long-term. Additionally, such boilers and turbines have high-temperature creep strength requirements in pressurized steam cycles. Superalloys in both wrought and cast forms are needed to replace ferritic-martensitic high strength steels and austenitic stainless steels to meet the long-term, high-temperature creep strength requirements in these pressurized steam cycles.

Superalloys, such as Ni-based superalloys, in both wrought and cast forms, are used to replace ferritic-martensitic high strength steels and austenitic stainless steels to meet the long-term, high-temperature creep strength requirements in these pressurized steam cycles.

IN740H is a boiler certified alloy, meeting component requirements for steam transfer and boiler pipes. IN740H has been used to manufacture boiler tubing, header and re-heater pipe as well as small fittings. The production of IN740H involves combinations of processes before fabrication into shape, such as vacuum induction melting (VIM), electroslag remelting (ESR) and/or vacuum arc remelting (VAR). While IN740H satisfies the performance requirements of A-USC designs in its wrought version, using the alloy in its cast form would be valuable in terms of range of component sizes, geometries and complexities, as well as cost.

Prior efforts made at producing articles of as-cast IN740H resulted in poor creep performance when compared to wrought IN740H articles. Several compositions within the nominal specified range for IN740H were investigated but failed to provide a material in the as-cast form that would withstand long-term, high-temperature exposure in creep.

In the future, advanced A-USC and/or sCO<sub>2</sub> power plant designs are expected to raise the efficiencies of coal-fired power plants from ~35 to >50%. It should be appreciated that improving the performance of the NiCrCoAlTi cast article over that of the existing conventionally cast versions of IN740 may provide as-cast material solutions that may withstand the higher operating temperatures found in advanced fossil energy power plants. A need exists in the art to develop a superalloy, such as a NiCrCoAlTi superalloy casting based on the nominal chemistry of INCONEL 740/

## 2

740H (IN740H). With operating temperatures of components in the coal-fired boiler and steam/CO<sub>2</sub> turbine greater than 760° C., Ni-based superalloys in both wrought and cast forms are needed to replace ferritic-martensitic high strength steels and austenitic stainless steels to meet the long-term, high-temperature creep strength requirements in these pressurized steam cycles.

**SUMMARY**

One object of at least one embodiment is related to a method of casting a creep-resistant Ni-based superalloy. The method includes forming a feed stock comprising Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B). The method further includes fabricating the creep-resistant Ni-based superalloy in a predetermined shape using the feed stock and at least one process comprising vacuum induction melting (VIM), electroslag remelting (ESR) and/or vacuum arc remelting (VAR).

One or more embodiments include the feed stock comprises at least Nickel (Ni) and Chromium (Cr).

One or more embodiments include melting the feed stock in a furnace, forming a liquid metal; pouring the liquid metal into a preheated mold, forming a molten metal; and solidifying the molten metal in the preheated mold, forming the creep-resistant Ni-based superalloy in the predetermined shape.

In one or more embodiments the feed stock is placed into a crucible inside the furnace, where the crucible may be a zirconia crucible inside the furnace and/or the furnace comprises a VIM furnace.

In one or more embodiments, the method includes melting the feed stock is carried out under vacuum and/or at a partial pressure between 50 and 400 Torr of Argon (Ar). Additionally, melting the metal Ni-based superalloy includes pouring the liquid metal into the mold when the temperature of the liquid metal is between 1 and 10 degrees Celsius above the melting temperature of the loaded feed stock.

In still other embodiments, the preheated mold is a graphite mold that is preheated to 500±200° C. (about 300° C. to about 700° C.) for a time ranging from about 10 minutes to about 5 hours. Additionally, the mold includes a zirconia wash coat.

Still another embodiment includes homogenizing the cast alloy including performing at least two of the sequential steps of treating the cast alloy between about 0.5 to about 5 hours at about 1050° C. to about 2000° C. (more specifically about 1075° C.); 1.5 to 3 hours at 1125±25° C.; 3 to 15 hours at 1200±25° C.; 3 to 24 hours at 1250±25° C.

In still other embodiments, the homogenized alloy is subjected to an aging heat treatment consisting of heating between about 4 to about 20 hours at about 800° C.;

Still another embodiment includes a method of casting a creep-resistant Ni-based superalloy, the method including loading the feed stock comprising Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B) into a crucible inside a VIM furnace. The method further includes melting the feed stock forming a liquid metal; pouring the liquid metal into a preheated mold in the VIM furnace, forming a molten

metal; and solidifying the molten metal in the preheated mold, forming the creep-resistant Ni-based superalloy in a predetermined shape.

Other embodiments relate to a method of casting a creep-resistant Ni-based superalloy. The method includes loading the feed stock into a crucible inside a VIM furnace, melting the feed stock forming a liquid metal, pouring the liquid metal into a preheated mold in the VIM furnace, forming a molten metal; and solidifying the molten metal forming an as-cast article of the creep-resistant Ni-based superalloy in a predetermined shape. The method includes the feed stock includes Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B). Melting the feed stock is performed in at least one of a vacuum and at a partial pressure between 50 and 400 Torr of Argon (Ar)

#### BRIEF DESCRIPTION OF THE DRAWINGS

The invention together with the above and other objects and advantages will be best understood from the following detailed description of the preferred embodiment of the invention shown in the accompanying drawings, wherein:

FIG. 1 depicts a representation of a conventional/prior art casting system;

FIG. 2 depicts a representation of a fine grain casting system in accordance with one embodiment, illustrating a melting step;

FIG. 3 depicts a representation of a fine grain casting system in accordance with one embodiment, illustrating a pouring step;

FIG. 4 depicts a representation of a fine grain casting system in accordance with one embodiment, illustrating a solidification step;

FIG. 5 depicts an end view of an ingot formed using prior art sectioned in half;

FIG. 6 depicts a side view of an ingot formed using prior art sectioned in half;

FIG. 7 depicts an image representing the macrostructure of a conventionally cast ingot sectioned in half;

FIG. 8 represents the macrostructure of an ingot formed using one embodiment of the present invention;

FIG. 9 depicts a graph illustrating creep properties of various ingots represented as data points on a Larson-Miller Parameter (LMP) plot and compared to the LMP curve for the wrought product;

FIG. 10 depicts a graph illustrating the comparison of creep tests at 259 MPa and 760° C. between conventional and FGH castings (present invention) in the form of creep strain as a function of creep life;

FIG. 11 depicts a graph illustrating results of tensile testing showing the ultimate tensile strength;

FIG. 12 depicts a graph illustrating results of tensile testing of 0.2% yield stress;

castings and the FGH casting (present invention) compared to data from wrought IN740H;

FIG. 14 depicts an image illustrating fracture of conventionally cast specimens in columnar region (L2B);

FIG. 15 depicts an image illustrating fracture of conventionally cast specimens in equiaxed region (L2LC);

FIG. 16 depicts an image illustrating fracture of a FGH cast specimen in accordance with one embodiment of the present invention;

FIG. 17 depicts a graph illustrating creep strength as a function of creep life during creep testing of L2B, L2C, and FGH at 760° C./259 MPa with L2B in the three different aging conditions; and

FIG. 18 depicts a graph illustrating creep strength as a function of creep life during creep testing of L2C (three specimens BI, FI, and H2) and FGH at 760° C./259 MPa.

#### DETAILED DESCRIPTION

The foregoing summary, as well as the following detailed description of certain embodiments of the present invention, will be better understood when read in conjunction with the appended drawings.

The following detailed description should be read with reference to the drawings in which similar elements in different drawings are numbered the same. The drawings, which are not necessarily to scale, depict illustrative embodiments and are not intended to limit the scope of the invention.

FIG. 1 depicts a representation of a known conventional casting system, generally designated 10. The system 10 includes a furnace 12, a VIM furnace for example, having a crucible 14. As depicted, furnace 12 further includes a mold 16, a graphite mold at room temperature, submerged in sand 18 on stand 20. The known casting system 10 illustrates superheat liquid 22, a 50° C. superheat liquid, that in poured into mold 16. The sand 18 cools the liquid in the mold 16 forming ingots.

One or more embodiments relates to a casting approach named Fine Grain Homogenized (FGH) to enable the use of a Ni-based superalloy, a NiCrCoAlTi superalloy for example, nominally based on IN740H, for cast articles in A-USC and sCO<sub>2</sub> power plants. The composition of the NiCrCoAlTi superalloy is within the limits (i.e., minimum-maximum) of IN740H listed in Table 1. In at least one embodiment, the FGH process is a fine-grain casting method which employs a low pouring temperature with pre-heated molds during VIM to refine the grain size of the as-cast solidified article. In addition to the physical development of a fine-grain cast structure in the article from the melt-solidification approach, a computationally optimized homogenization technique specifically designed for the NiCrCoAlTi superalloy is also utilized to ensure homogeneous chemical distribution of the hard to diffuse elements of this chemistry throughout the as-cast article.

TABLE 1

| Element | Cr   | Co   | Al   | Ti   | Nb  | Fe   | C     | Mn  | Mo   | Si  | Cu     | P    | s    | B      | NI   |
|---------|------|------|------|------|-----|------|-------|-----|------|-----|--------|------|------|--------|------|
| Minimum | 23.5 | 15.0 | 0.2  | 0.5  | 0.5 | —    | 0.005 | —   | —    | —   | —      | —    | —    | 0.0006 | Bal. |
| Nominal | 24.5 | 20   | 1.35 | 1.35 | 1.5 | 0.03 | —     | 0.1 | 0.15 | —   | —      | —    | —    | —      | —    |
| Maximum | 25.5 | 22.0 | 2.0  | 2.5  | 2.5 | 3.0  | 0.08  | 1.0 | 2.0  | 1.0 | a.s.o. | 0.03 | 0.03 | 0.006  | —    |

FIG. 13 depicts a graph illustrating results of tensile testing showing the elongation to failure of all conventional

65 In according to one embodiment, the constituent elements of an alloy are combined using high-purity, industrial-grade

metal/alloy for a solidified article target mass of ~7 kg (although article size is not a constraining condition). Chromium may be added as part of master alloys consisting of Ni-25Cr, Ni-30Co-30Cr and/or Ni-30Cr in order to reduce the overall oxygen concentration in the alloys as the raw Cr used for alloy manufacture contained 5200 ppm oxygen. The master alloys were previously melted using a two-step process of VIM followed by ESR to obtain ~68 kg ingots (again, article size is not a constraining condition). This results in a reduction in oxygen concentration and sulfur concentration by reducing the density of non-metallic inclusions. It should be appreciated that various starting material combinations may be used as feed stock for embodiments of the invention and are again not a constraining condition.

The feed stock materials constituting the Ni-based superalloy, NiCrCoAlTi superalloy for example, are loaded in a crucible, a zirconia crucible for example, inside a vacuum induction furnace (VIM). The liquid metal was subsequently poured into a graphite mold to solidify as a cylinder 100 mm in diameter for example. To limit excess carbon pickup in the mold, a zirconia wash coat was used in the mold as a barrier between the liquid metal and the graphite mold walls. The mold was preheated to 500° C. prior to being placed in the VIM furnace. To maintain mold temperature, the graphite mold with zirconia wash coat was wrapped in fiberglass insulation to slow the cooling rate of the mold.

Pouring was initiated when the liquid metal was thoroughly molten and a few degrees above the NiCrCoAlTi superalloy melting temperature as determined by visually observing the viscosity of the liquid and color of the melt pool.

The as-cast article was homogenized in a vacuum heat treatment furnace using a computationally optimized homogenization heat treatment cycle. The homogenization cycle leads to a controlled and random dispersal of the alloy constituents that significantly reduces chemical segregation within the as-cast article. The homogenization heat treatment for the NiCrCoAlTi superalloy leads to specific element segregation below ±1% variation from the nominal chemistry of these elements throughout the article. For the NiCrCoAlTi superalloy casting, the cycle sequence includes about 1 hour at about 1075° C.+about 3 hours at about 1125° C.+about 8 hours at about 1200° C.+about 8 hours at about 1250° C. is used.

The as-homogenized article was subjected to an aging heat treatment consisting of 16 hours at 800° C.

One or more embodiments includes a homogenization heat treatment based on the scale of the microstructure which is dependent upon the thickness of the cast article. The preferred embodiment incorporates a heat treatment to limit residual inhomogeneity to <10%, or more preferable to <5% or more preferable to <1% as described in TABLES 2 and 3. Furthermore, it should be appreciated that commercial heat treatment facilities may be limited to the maximum temperature available. Typical maximum temperatures are 1200° C. and 1250° C. Table X describes treatments at both of these maximum temperatures.

TABLE 2

| Section Size | Maximum Temperature 1250° C. |               |               |
|--------------|------------------------------|---------------|---------------|
|              | <10%                         | <5%           | <1%           |
| Up to 5 in   | 1075 C./1 h +                | 1075 C./1 h + | 1075 C./1 h + |
|              | 1125 C./3 h +                | 1125 C./3 h + | 1125 C./3 h + |
|              | 1200 C./6 h                  | 1200 C./8 h   | 1200 C./8 h   |
|              |                              | 1250 C./8 h   | 1250 C./12 h  |
|              |                              |               | 1250 C./24 h  |
|              |                              | 1075 C./1 h + | 1075 C./1 h + |

TABLE 2-continued

| Section Size | Maximum Temperature 1250° C. |               |               |
|--------------|------------------------------|---------------|---------------|
|              | <10%                         | <5%           | <1%           |
| >8 inch      | 1075 C./1 h +                | 1075 C./1 h + | 1075 C./1 h + |
|              | 1125 C./6 h +                | 1125 C./6 h + | 1125 C./6 h + |
|              | 1200 C./8 h +                | 1200 C./8 h + | 1200 C./8 h + |
|              |                              | 1250 C./16 h  | 1250 C./26 h  |
|              |                              |               | 1250 C./50 h  |
|              |                              |               |               |

TABLE 3

| Section Size | Maximum Temperature 1200° C. |               |               |
|--------------|------------------------------|---------------|---------------|
|              | <10%                         | <5%           | <1%           |
| Up to 5in    | 1075 C./1 h +                | 1075 C./1 h + | 1075 C./1 h + |
|              | 1125 C./3 h +                | 1125 C./3 h + | 1125 C./3 h + |
|              | 1200 C./6 h                  | 1200 C./8 h   | 1200 C./30 h  |
|              | 1075 C./1 h +                | 1075 C./1 h + | 1075 C./1 h + |
|              | 1125 C./3 h +                | 1125 C./3 h + | 1125 C./3 h + |
|              | 1200 C./24 h                 | 1200 C./36 h  | 1200 C./65 h  |
| >8 inch      | 1075 C./1 h +                | 1075 C./1 h + | 1075 C./1 h + |
|              | 1125 C./6 h +                | 1125 C./6 h + | 1125 C./6 h + |
|              | 1200 C./40 h                 | 1200 C./60 h  | 1200 C./110 h |

FIG. 2 depicts a representation of a fine grain casting system, generally designated 100, in accordance with one embodiment. FIG. 2 specifically depicts the melting step. The system 100 includes a furnace 112, a VIM furnace for example, defining a vacuum chamber 124 having a crucible 114. In the illustrated embodiment, the crucible 114 is positioned in a melt box 115 where it is wrapped in a sleeve 128 including induction coils 126.

As depicted, furnace 112 further includes a mold 116, a graphite mold, wrapped in insulation 118, fiberglass insulation for example, on stand 120. The system 100 illustrates liquid metal 122, adaptable to be poured into mold 116.

FIG. 3 the fine grain casting system 100 in accordance with one embodiment, illustrating a pouring step. FIG. 4 depicts a representation of a fine grain casting system 100 illustrating a solidification step forming ingot 132.

In one or more embodiments feed stock materials constituting a Ni-based superalloy, a NiCrCoAlTi superalloy for example, are cast into the Ni-based superalloy of predetermined shape, an ingot with for example, using the system 100. In one or more embodiments, the feed stock comprises Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B). In one embodiment, the feed stock comprises Nickel (Ni) and Chromium (Cr).

The feed stock is loaded in the crucible 114, a zirconia crucible, inside the furnace 112, a vacuum induction furnace or VIM for example, forming a loaded feed stock. The feed stock melts in the furnace 112, forming a liquid metal 122.

The liquid metal 122 is poured into a graphite mold 116 to solidify (as a cylinder 100 mm in diameter for example). To limit excess carbon pickup in the mold, a zirconia wash coat 130 was used in the mold 116 as a barrier between the liquid metal and the graphite mold walls. The mold 116 was preheated to 500° C. prior to being placed in the VIM furnace. To maintain mold temperature, the graphite mold

**116** with zirconia wash coat **130** was wrapped in fiberglass insulation **118** to slow the cooling rate of the mold.

One or more embodiments described herein includes a method of casting a creep-resistant Ni-based superalloy. The method includes forming a feed stock and fabricating an as-cast article comprising creep-resistant Ni-based superalloy in a predetermined shape. The feed stock includes Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B). fabricating an as-cast article includes using the feed stock and at least one process comprising vacuum induction melting (VIM), electroslag remelting (ESR) and/or vacuum arc remelting (VAR). In at least one embodiment, the feed stock comprises at least Nickel (Ni) and Chromium (Cr).

One embodiment includes melting the feed stock in a furnace, forming a liquid metal, pouring the liquid metal into a preheated mold, forming a molten metal; and solidifying the molten metal in the preheated mold, forming the as-cast article.

One or more embodiments includes homogenizing the as-cast article in a vacuum heat treatment furnace using a computationally optimized homogenization heat treatment cycle, forming a controlled and random dispersal of alloy constituents that significantly reduces chemical segregation within the as-cast article. Homogenizing the as-cast article forms a specific element segregation below  $\pm 1\%$  variation from the nominal chemistry of these elements throughout the as-cast article. Homogenizing the as-cast article may include a sequence of heating or treatment including one hour at about 1075° C., three hours at about 1125° C., eight hours at about 1200° C. and eight hours at about 1250° C.

In one or more embodiments, melting the feed stock is carried out in at least one of a vacuum and at a partial pressure between 50 and 400 Torr of Argon (Ar). Additionally, melting the metal Ni-based superalloy may include pouring the liquid metal into the crucible when the temperature of the liquid metal is between 1 and 10 degrees Celsius above the melting temperature of the loaded feed stock.

Preheating the mold may include heating the mold from between about 300° C. to about 700° C. from about 10 minutes to about 5 hours.

In one or more embodiments, the cast alloy is subjected to a homogenization heat treatment comprising at least two of the sequential steps of treating the cast alloy: 0.5 to 5

FIG. 5 depicts an end view of an ingot 200 sectioned in half formed using conventional techniques. FIG. 5 depicts the ingot 200 a large columnar zone 210 that transitions to an equiaxed grain structure zone 212. FIG. 6 depicts an elevational view of an ingot 300 sectioned in half formed using conventional techniques similar to that of ingot 300.

FIGS. 7 and 8 represent the macrostructure of conventional and FGH ingots sectioned in half. FIG. 7 illustrates the typical macrostructure of a conventionally cast ingot. A small chill zone appears on the sides and bottom where the liquid metal first contacted the mold. A large columnar zone is observed next that transitions to an equiaxed grain structure in the middle of the ingot. FIG. 8 illustrates the macrostructure of an ingot formed using one or more embodiments of the present invention (referred to as a FGH article). In FIG. 8, the chill zone was reduced and, more importantly, the columnar zone was significantly reduced in thickness (and volume) in comparison to the conventional cg. This results in most of the as-cast article having a more desirable fine-grained equiaxed microstructure. Moreover, the grain size in the equiaxed region was considerably reduced in comparison to the conventional casting. This approach resulted in a grain structure that was considerably more homogeneous physically and as chemically compared to the conventional casting.

TABLE 4 illustrates the composition of castings from XRF Analysis (wt. %). Tensile and creep testing were systematically performed on these articles as well as for the FGH article following homogenization and aging heat treatments. Six (6) conventional castings were selected for inclusion in TABLE 4 for comparison to the FGH article. It should be noted that the conventional castings were also homogenized using the same computationally optimized heat treatment schedule as was used for the FGH article.

While the standard aging treatment consisted of 16 hours at 800° C. Two additional aging heat treatments were investigated for alloys L2B, L2C and L2LC. The first alternate aging heat treatment consisted of heating the ingots to 850° C. for 4 hours followed by lowering the temperature to 800° C. for an additional 8 hours. These aged articles were then allowed to cool to room temperature in air. The second alternate aging heat treatment was to soak the as-cast (and homogenized) articles at 950° C. for 2 hours followed by 8 hours at 800° C. Following the aging cycle, the articles were once again cooled to room temperature in air. It should be appreciated that conventionally cast articles B, L1B and L2B contained La. This was used to reduce the S content.

TABLE 4

|      | Ni   | Cr   | Co   | Al   | Ti   | Nb   | Fe   | C*   | Mn   | Mo  | Si   | B**    | La    |
|------|------|------|------|------|------|------|------|------|------|-----|------|--------|-------|
| B    | Bal. | 24.8 | 19.6 | 1.24 | 1.33 | 1.49 | 2.47 | 0.03 | 0.31 | 0.5 | 0.14 |        | ~0.01 |
| L1B  | Bal. | 23.7 | 17.9 | 0.74 | 1.12 | 1.30 | —    | 0.03 | 0.10 | 2.0 | 0.07 | 0.0010 | 0.023 |
| L2B  | Bal. | 24.1 | 16.4 | 1.03 | 1.49 | 1.30 | —    | 0.03 | 0.11 | 2.0 | 0.06 | 0.0008 | 0.023 |
| L2C  | Bal. | 23.8 | 18.2 | 1.14 | 1.48 | 1.29 | 0.64 | 0.03 | 0.10 | 2.0 | 0.18 | 0.0050 | —     |
| L2LC | Bal. | 23.6 | 18.0 | 1.03 | 1.52 | 1.30 | 0.08 | 0.02 | 0.10 | 2.0 | 0.05 | 0.0006 | —     |
| L3   | Bal. | 24.1 | 20.2 | 1.40 | 2.49 | 0.49 | —    | 0.03 | 0.10 | 2.0 | 0.07 | 0.0011 | —     |
| FGH  | Bal. | 24.4 | 19.6 | 1.15 | 1.53 | 1.58 | —    | 0.03 | 0.32 | 0.5 | 0.21 | 0.0011 | —     |

hours at  $1075 \pm 25^\circ \text{ C.}$ ; 1.5 to 3 hours at  $1125 \pm 25^\circ \text{ C.}$ ; 3 to 15 hours at  $1200 \pm 25^\circ \text{ C.}$ ; 3 to 24 hours at  $1250 \pm 25^\circ \text{ C.}$  The cast alloy is characterizable by a level of chemical homogeneity, defined as variations between local and nominal chemistry following homogenizing and measured using wavelength dispersive x-ray fluorescence, of less than  $\pm 1\%$ , or less than  $\pm 2\%$ , or less than  $\pm 5\%$ .

Table 5 compiles various measurements obtained from the macrostructures illustrated in FIGS. 7 and 8. The conventional casting approach for these alloys resulted in the commonly observed macrostructure zone ratio seen in FIG. 7. The chill zone width was limited to approximately 2 mm. A large, columnar zone next formed, which was approximately 21 mm in thickness, as measured from each surface of the mold. The last region to form was the central equiaxed

zone spanning a radius of 27 mm from the cylindrical article centerline. This zone started ~23 mm from the bottom mold surface.

In FIG. 8, the equiaxed zone of the FGH casting was significantly greater than that in the conventional casting. The equiaxed zone extended from about 48 mm from the centerline of the cylindrical article with the chill/columnar zone ~4 mm from the mold bottom surface. Both the columnar and chill zone thicknesses were greatly reduced, i.e., 3 mm for the columnar zone and 0.6 mm for the chill zone, representing an 86% and 72% reduction, respectively, from the average of the conventional cast articles.

The average grain size in the equiaxed regions were calculated to be  $717 \pm 101 \mu\text{m}$  for the conventionally as-cast articles as compared to  $289 \pm 42 \mu\text{m}$  for the FGH as-cast article. Overall, the grain size was significantly more homogeneous (i.e., the physical grain structure) in the FGH as-cast article than in the conventionally as-cast article, which had grain sizes ranging from approximately  $40 \mu\text{m}$  to greater than  $4,000 \mu\text{m}$ .

TABLE 5

|                                                             | Conventional Casting | Fine-Grain Casting |
|-------------------------------------------------------------|----------------------|--------------------|
| We: Equiaxed Width (mm)*                                    | $27.1 \pm 1.2$       | $48.1 \pm 0.4$     |
| Wc: Columnar Width (mm)*                                    | $20.8 \pm 1.0$       | $2.9 \pm 0.3$      |
| Wch: Chill Zone Width (mm)*                                 | $2.0 \pm 0.7$        | $0.6 \pm 0.1$      |
| Average Grain Size in the Equiaxed Zone ( $\mu\text{m}$ )** | $717 \pm 101$        | $289 \pm 42$       |

\*Standard deviations reported over 12 equally spaced measurements along the ingot centerline.

\*\*Standard deviations reported over 8 randomly drawn lines (linear intersect technique).

FIG. 9 depicts the creep properties of the various ingots represented as data points on a Larson-Miller Parameter (LMP) and are compared to the LMP curve for the wrought product, IN740H, (i.e., solid line representing a trendline of the wrought data) at  $775^\circ \text{C}$ . Various specimens were tested from six (6) of the castings listed in TABLE 4 under different stresses and temperatures. For convenience, the creep results (with additional information) are also listed in TABLE 6. Data from the conventional castings show significant scatter with data points predominantly located to the left of the IN740H mean LMP trendline curve. Alloy L2B appeared to outperform the other conventional castings with the exception of the  $760^\circ \text{C}/259 \text{ MPa}$  creep test. It should be noted that the scatter was also present when testing the same alloy under identical conditions, as shown in TABLE 6 where three specimens from L2C were tested at  $760^\circ \text{C}/259 \text{ MPa}$ . The results show times to failure of 250, 575 and 1069 hours. The two-step aging heat treatment increased the times to failure when compared to the standard aging treatment, particularly for alloys L2B and L2LC.

The FGH articles were tested under six (6) different stresses and two temperatures to obtain an LMP curve (data points in FIG. 9) and ensure statistical evidence when reporting the creep properties. Two different temperatures were considered, and the full list of testing parameters are shown in TABLE 6.

The data for the six (6) tests fall on the wrought curve, or just slightly beyond it. The shortest test was performed at  $790^\circ \text{C}/233 \text{ MPa}$  and lasted 536 hours while the longest test was obtained at  $760^\circ \text{C}/207 \text{ MPa}$  which lasted 12,732 hours.

TABLE 6

| 5  | Alloy      | Temperature ( $^\circ \text{C}$ ) | Stress (MPa) | Time to Failure (h) | LMP           |                           |
|----|------------|-----------------------------------|--------------|---------------------|---------------|---------------------------|
|    |            |                                   |              |                     | (C = 20)/1000 | Elongation to Failure (%) |
| 10 | B          | 735                               | 310          | 103                 | 22.19         | 0.2                       |
|    |            | 760                               | 259          | 446                 | 23.40         | 2.9                       |
|    |            | 785                               | 207          | 555                 | 24.06         | 1.0                       |
|    | LIB        | 775                               | 207          | 169                 | 23.29         | 1.9                       |
|    |            | 800                               | 276          | 93                  | 23.57         | 5.2                       |
|    | L2B        | 760                               | 259          | 94                  | 22.70         | 2.7                       |
|    |            | 775                               | 207          | 1,739               | 24.36         | 2.1                       |
|    |            | 790                               | 155          | 1,855               | 24.73         | 1.5                       |
| 15 | L2B*       | 760                               | 259          | 966                 | 23.74         | 2.4                       |
|    |            | 760                               | 259          | 954                 | 23.74         | 2.2                       |
|    | L2C        | 760                               | 259          | 250                 | 23.14         | 2.2                       |
|    |            | 760                               | 259          | 575                 | 23.51         | 2.1                       |
|    | L2C*       | 760                               | 259          | 1,069               | 23.79         | 1.7                       |
|    |            | 760                               | 259          | 907                 | 23.72         | 3.7                       |
| 20 | L2C**      | 760                               | 259          | 685                 | 23.59         | 6.4                       |
|    |            | 760                               | 259          | 15                  | 21.87         | 0.04                      |
|    | L2LC       | 760                               | 259          | 95                  | 22.70         | 0.04                      |
|    |            | 760                               | 259          | 112                 | 22.78         | 0.08                      |
|    | FGH        | 760                               | 259          | 1,479               | 23.93         | 1.4                       |
|    |            | 790                               | 233          | 536                 | 24.16         | 1.6                       |
|    | 760/790*** | 760                               | 207          | 4,806               | 24.46         | 0.92                      |
|    |            | 790                               | 181          | 2,845               | 24.93         | 0.95                      |
|    |            | 760/790***                        | 155          | 4,571               | 25.15         | 0.35                      |
|    |            | 790                               | 129          | 12,732              | 25.62         | 1.3                       |

\*Aged using the 2-step heat treatment  $850^\circ \text{C}$ . for 4 hours followed by  $800^\circ \text{C}$ . for 8 hours.

\*\*Aged using the 2-step heat treatment  $950^\circ \text{C}$ . for 2 hours followed by  $800^\circ \text{C}$ . for 8 hours.

\*\*\*Test started at  $760^\circ \text{C}$ ., stopped after 8,896 hours and restarted at  $790^\circ \text{C}$ . to accelerate.

30 A comparison of the creep tests at 259 MPa and  $760^\circ \text{C}$ . between the conventional and the FGH castings is shown in the graph illustrated in FIG. 10 in the form of creep strain as a function of creep life. The average results for all conventional castings resulted in a value of elongation to failure in creep of approximately 1.4% with a creep life of 489 hours. Comparatively, while the elongation to failure in creep for the FGH casting remains relatively the same, the increase in creep life is significantly greater, reaching 1,479 hours, a more than three-fold increase of the average of all conventional castings. Meanwhile, the best performing conventionally cast specimen (i.e., in terms of creep life) reached a slightly higher value for elongation to failure in creep of 1.7%. However, the time to failure, while high for the conventionally cast ingots, remained lower at 1,069 hours. The creep life of the FGH cast material still outperformed the best conventionally cast specimen by 38%.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155

Results of the 0.2% yield stress (YS) shown in FIG. 12 reveal values of the FGH cast articles close to the wrought alloy and significantly greater than those conventionally cast. For instance, at room temperature the average YS of conventionally cast articles was  $491 \pm 76$  MPa, and ranged from 390 MPa for L1B to 605 MPa for L3. Alternatively, the average YS of FGH cast articles was  $668 \pm 4$  MPa. At elevated temperature, the YS of the FGH cast articles was similar to that of the wrought alloy. Average values at  $800^\circ$  C. are  $545 \pm 6$  MPa for the FGH cast samples and  $418 \pm 62$  MPa for the conventionally cast samples. Only alloy L3 reached a YS close to that of the FGH cast material with an average of  $519 \pm 6$  MPa.

Unlike the UTS and YS, the elongation to failure of the FGH cast articles was between values measured on the specimens from the conventional castings, FIG. 13. At room temperature, the average elongation to failure was similar at  $11 \pm 7\%$  and  $12 \pm 2\%$  for the conventional and FGH castings, respectively. However, and as the standard deviations suggest, the range for the conventional castings spanned quite a large span in elongation to failure, ranging from 3% to 21%. The latter value is close to the elongation to failure of the wrought product at 24%. Similar trends were observed at elevated temperatures with the average elongation to failure of  $10 \pm 8\%$  and  $6 \pm 1\%$  for the conventional and FGH castings at  $800^\circ$  C., respectively. Alloy L1B exhibited an average elongation to failure of  $24 \pm 6\%$ , which is similar to that of the wrought product.

TABLE 7

| Alloy | Temperature (C.) | UTS (MPa) | 0.2% Yield Stress (MPa) | Elongation to Failure (%) |
|-------|------------------|-----------|-------------------------|---------------------------|
| B     | 800              | 525       | 426                     | 6.0                       |
|       | 800              | 520       | 421                     | 7.0                       |
| LIB   | 24               | 574       | 417                     | 17.7                      |
|       | 24               | 425       | 390                     | 3.0                       |
|       | 24               | 602       | 431                     | 17.0                      |
|       | 24               | 587       | 439                     | 14.8                      |
|       | 24               | 617       | 435                     | 18.3                      |
|       | 750              | 557       | 352                     | 27.3                      |
|       | 750              | 527       | 354                     | 12.5                      |
| L2B   | 800              | 461       | 327                     | 20.0                      |
|       | 800              | 458       | 322                     | 28.0                      |
|       | 24               | 643       | 523                     | 8.3                       |
|       | 750              | 495       | 424                     | 9.4                       |
|       | 750              | 662       | 451                     | 14.0                      |
| L2B*  | 800              | 578       | 424                     | 11.0                      |
|       | 800              | 558       | 411                     | 14.9                      |
|       | 24               | 669       | 535                     | 6.1                       |
| L2B** | 800              | 554       | 400                     | 8.2                       |
|       | 800              | 560       | 407                     | 8.7                       |
|       | 24               | 724       | 528                     | 15.0                      |
| L2C   | 800              | 495       | 405                     | 5.2                       |
|       | 800              | 502       | 406                     | 4.6                       |
|       | 24               | 581       | 543                     | 2.8                       |
|       | 24               | 566       | 548                     | 5.2                       |
|       | 200              | 550       | 496                     | 8.3                       |
|       | 200              | 539       | 492                     | 5.3                       |
|       | 400              | 573       | 497                     | 9.5                       |
|       | 400              | 520       | 453                     | 14.8                      |
|       | 600              | 127       | 467                     | 5.9                       |
|       | 600              | 500       | 425                     | 9.3                       |
| L2C*  | 650              | 517       | 420                     | 12.6                      |
|       | 650              | 556       | 461                     | 6.4                       |
|       | 700              | 285       | 436                     | 8.6                       |
|       | 700              | 495       | 412                     | 14.3                      |
|       | 750              | 480       | 443                     | 7.8                       |
|       | 750              | 501       | 455                     | 8.9                       |
|       | 800              | 562       | 419                     | 11.6                      |
|       | 800              | 490       | 391                     | 10.5                      |
|       | 24               | 552       | 509                     | 3.7                       |
|       | 800              | 581       | 427                     | 6.4                       |

TABLE 7-continued

| Alloy | Temperature (C.) | UTS (MPa) | 0.2% Yield Stress (MPa) | Elongation to Failure (%) |
|-------|------------------|-----------|-------------------------|---------------------------|
| L2C** | 24               | 654       | 557                     | 9.4                       |
|       | 800              | 458       | 408                     | 4.3                       |
|       | 24               | 819       | 577                     | 21.3                      |
|       | 800              | 478       | 424                     | 1.6                       |
| L2LC* | 24               | 775       | 566                     | 14.3                      |

\*Aged using the 2-step heat treatment  $850^\circ$  C./4 h +  $800^\circ$  C./8 h.

\*\*Aged using the 2-step heat treatment  $950^\circ$  C./2 h +  $800^\circ$  C./8 h.

Fracture surfaces of selected cast alloys are shown in FIGS. 14-16. These images represent three types of general fracture observed. FIG. 14 illustrates failure of a specimen extracted from the columnar region of a conventional casting (L2B) while FIG. 15 is representative of failure of a specimen from the equiaxed region of the conventional castings (L2LC pictured). A fracture surface of the FGH casting is shown in FIG. 16 revealing the finer grain structure of the alloy. Overall, fracture analysis showed predominantly intergranular failure, particularly for specimens tested in the equiaxed region of the conventional castings. The FGH casting, however, showed evidence of limited ductility.

FIG. 17 depicts a graph illustrating creep strain rate as a function of time during creep testing of L2B, L2C, and FGH at  $760^\circ$  C./259 MPa with L2B in the three different aging conditions. FIG. 18 depicts a graph illustrating creep strain as a function of time during creep testing of L2C (three specimens B1, F1, and H2) and FGH at  $760^\circ$  C./259 MPa.

The FGH casting performed better than the other conventional castings in terms of YS and UTS with values of YS close to that of the wrought product. A primary reason is the finer grain size in the FGH casting (Hall-Petch effect). The Hall-Petch effect is well known. That is YS and UTS vary inversely as a function of grain size with fine grained metals and alloys having higher YS and UTS compared to larger grained metals and alloys. However, fine grained metals and alloys typically have poor creep life compared to metals and alloys with larger grain sizes. This is not the case for the FGH articles, which is an unexpected result.

The FGH articles have long creep lives compared to the larger grained conventionally cast articles. This behavior is associated directly with carbide morphology and carbide distribution. In the FGH articles, carbides are uniformly distributed throughout the microstructure with few regions devoid of carbide. In addition, the carbides are blocky in the FGH articles whereas in the conventionally cast articles, the carbides are absent over long stretches of grain boundary length, or are thin/elongated and/or continuous, or are cellular in nature, or are a combination of these. The FGH casting approach not only changes the proportion of equiaxed to columnar zones but also changes the grain size within these zones. In doing so, the FGH approach also changes the morphology and distribution of carbides. These combined effects not only improve the tensile strength of the FGH as-cast articles but also improve creep performance as measured by the LMP (as a direct result of longer creep life).

An alternative casting approach, FGH, combines fine-grain casting techniques and computational homogenization heat treatment to improve the creep life of NiCrCoAlTi (Ni-based) superalloy (based on the nominal composition range of IN740H). This approach promotes a homogeneous physical grain structure, grain boundary precipitate repartition, and enhanced chemical homogeneity within the cast and heat-treated article. The LMP values of the FGH NiCr-CoAlTi (Ni-based) superalloy cast article matched, or slightly surpassed those reported for wrought IN740H.

The macrostructure of the FGH cast articles consisted of a primary equiaxed zone and much reduced chill/columnar zones. These zones were minimized by the rapid solidification rate of the molten alloy as consequences of the low pouring superheat and the heated mold. The average grain size in the equiaxed region was considerably reduced in the FGH cast articles.

The refined grain size of the FGH cast articles led to an increased density of nucleation sites for  $M_{23}C_6$ , grain boundary carbides, and thus, an overall reduction in carbide thickness. This alternative approach reduced discrepancies in their repartition of carbides along the grain boundaries as well as changing the carbide morphology, leading to reduced regions of no carbide precipitation and localized stress concentrations.

Intricate grain boundaries in the FGH cast articles were developed when compared to relatively straight, or minimally curved, grain boundaries typical of the conventionally cast articles. This change in general morphological feature directly contributed to improved creep life as crack propagation was tempered by the tortuous nature of the path with enhanced opportunities for crack wedging.

The YS and UTS of the FGH cast articles were improved when compared to conventionally cast ones. The FGH cast articles values were close to the YS and UTS values reported for wrought IN740H. Changes in chemistry within the range reported for IN740H resulted in relatively considerable differences in YS, UTS, and elongation to failure in the conventional castings. Thus, further improvement in the properties of the FGH casting can be considered with respect to overall chemistry and compositional range.

The composition of the NiCrCoAlTi (Ni-based) superalloy can be varied within the range of commercial IN740H as specified in TABLE 1.

The homogenization heat treatment used in the making of the FGH as-cast article described herein was optimized using computational design. However, other combinations of time/temperature and number of segments can be utilized but ultimately must achieve the same level of homogenization (i.e.,  $\pm 1\%$  of nominal, herein, or better) in order to maintain tensile and creep performance, i.e., high YS and creep life as measured by LMP.

As an example, aging trials on IN740H were performed and revealed variations in the size or fraction of precipitate phases such as  $\gamma'$  and carbides ( $MC$  and  $M_{23}C_6$ ). Therefore, the aging heat treatment can also be targeted for specific properties. Aging can be performed using a single-step heat treatment (time and temperature) or a multi-step heat treatment, consisting of two or more aging temperatures with various holding times. The selection of such corresponds with the desire to achieve a particular set of microstructural features necessary to optimize a particular property (e.g., yield stress, creep life, fatigue life, oxidation resistance, etc.).

The superheat temperature (of the liquid metal prior to pouring) can be varied as well as the cooling rate determined by the temperature of the liquid metal and the temperature of the mold. The mold can be either pre-heated or heated in the furnace. Various temperatures can be employed. Ultimately, they must achieve a mostly equiaxed and refined grain structure in the cast ingot. A combination of possibilities exists each one resulting in a set of microstructural features that would affect strength and creep life. The approach outlined herein describes one that produced a fine-grained physical microstructure (casting approach) with a very high degree of chemical homogeneity (homogenization cycle) which subsequently yielded an as-cast article

with high YS (based on the fine-grained nature of the microstructure) and long creep life (based on chemical homogeneity and carbide morphology and distribution).

Control cooling techniques also present many possibilities, utilizing either a controlled cooling rate from solution heat treatment temperature or modifying the aging heat treatment approach. That is, varying the temperature (or room temperature prior to aging), and the time at temperature, can be used to control the size and distribution of grain boundary precipitates. Many such possibilities can be explored to modify the mechanical behaviors described herein or to address other property concerns like fatigue life or oxidation resistance.

Having described the basic concept of the embodiments, it will be apparent to those skilled in the art that the foregoing detailed disclosure is intended to be presented by way of example. Accordingly, these terms should be interpreted as indicating that insubstantial or inconsequential modifications or alterations and various improvements of the subject matter described and claimed are considered to be within the scope of the spirited embodiments as recited in the appended claims. Additionally, the recited order of the elements or sequences, or the use of numbers, letters or other designations therefor, is not intended to limit the claimed processes to any order except as may be specified. All ranges disclosed herein also encompass any and all possible sub-ranges and combinations of sub-ranges thereof. Any listed range is easily recognized as sufficiently describing and enabling the same range being broken down into at least equal halves, thirds, quarters, fifths, tenths, etc. As a non-limiting example, each range discussed herein can be readily broken down into a lower third, middle third and upper third, etc. As will also be understood by one skilled in the art all language such as up to, at least, greater than, less than, and the like refer to ranges which are subsequently broken down into sub-ranges as discussed above. As utilized herein, the terms "about," "substantially," and other similar terms are intended to have a broad meaning in conjunction with the common and accepted usage by those having ordinary skill in the art to which the subject matter of this disclosure pertains. As utilized herein, the term "approximately equal to" shall carry the meaning of being within 15, 10, 5, 4, 3, 2, or 1 percent of the subject measurement, item, unit, or concentration, with preference given to the percent variance. It should be understood by those of skill in the art who review this disclosure that these terms are intended to allow a description of certain features described and claimed without restricting the scope of these features to the exact numerical ranges provided. Accordingly, the embodiments are limited only by the following claims and equivalents thereto. All publications and patent documents cited in this application are incorporated by reference in their entirety for all purposes to the same extent as if each individual publication or patent document were so individually denoted.

All numeric values are herein assumed to be modified by the term "about", whether or not explicitly indicated. The term "about" generally refers to a range of numbers that one of skill in the art would consider equivalent to the recited value (e.g., having the same function or result). In many instances, the terms "about" may include numbers that are rounded to the nearest significant figure.

The recitation of numerical ranges by endpoints includes all numbers within that range (e.g., 1 to 5 includes 1, 1.5, 2, 2.75, 3, 3.80, 4, and 5).

One skilled in the art will also readily recognize that where members are grouped together in a common manner, such as in a Markush group, the present invention encom-

## 15

passes not only the entire group listed as a whole, but each member of the group individually and all possible subgroups of the main group. Accordingly, for all purposes, the present invention encompasses not only the main group, but also the main group absent one or more of the group members. The present invention also envisages the explicit exclusion of one or more of any of the group members in the claimed invention.

What is claimed is:

1. A method of casting a creep-resistant Ni-based superalloy, the method comprising:

forming a feed stock comprising Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B);

20 fabricating an as-cast article comprising creep-resistant Ni-based superalloy in a predetermined shape using the feed stock and at least one process comprising vacuum induction melting (VIM), electroslag remelting (ESR) and/or vacuum arc remelting (VAR); and homogenizing the as-cast article, wherein homogenizing the as-cast article comprises a heating sequence of one hour at about 1075° C., three hours at about 1125° C., eight hours at about 1200° C. and eight hours at about 1250° C.

2. The method of claim 1, wherein the feed stock comprises at least Nickel (Ni) and Chromium (Cr).

3. The method of claim 1 wherein fabricating the creep-resistant Ni-based superalloy comprises:

melting the feed stock in a furnace, forming a liquid metal;

pouring the liquid metal into a preheated mold, forming a molten metal; and

solidifying the molten metal in the preheated mold, forming the as-cast article.

4. The method of claim 3 wherein homogenizing the as-cast article further comprises forming a controlled and random dispersal of alloy constituents that reduces chemical segregation within the as-cast article.

5. The method of claim 4 wherein the homogenizing the as-cast article forms a specific element segregation below  $\pm 1\%$  variation from the nominal chemistry of these elements throughout the as-cast article.

6. The method of claim 4 further comprises loading the feed stock into a crucible inside the furnace.

7. The method of claim 6 further comprises loading the feed stock into a zirconia crucible inside the furnace, forming a loaded feedstock.

8. The method of claim 3 wherein the furnace comprises a VIM furnace.

9. The method of claim 3 wherein melting the feed stock is carried out in at least one of a vacuum and at a partial pressure between 50 and 400 Torr of Argon (Ar).

10. The method of claim 3 wherein melting the metal Ni-based superalloy includes pouring the liquid metal into the preheated mold when the temperature of the liquid metal is between 1 and 10 degrees Celsius above the melting temperature of the loaded feed stock.

11. The method of claim 3 wherein the preheated mold is a graphite mold.

12. The method of claim 3 wherein the preheated mold includes a zirconia washcoat and is preheated prior to being placed in the furnace.

## 16

13. The method of claim 3 wherein the preheated mold is heated to about 300° C. to about 700° C. from about 10 minutes to about 5 hours.

14. The method of claim 1 wherein the as-cast article is characterizable by a level of chemical homogeneity, defined as variations between local and nominal chemistry following homogenizing and measured using wavelength dispersive x-ray fluorescence, of less than  $\pm 1\%$ , or less than  $\pm 2\%$ , or less than  $\pm 5\%$ .

15. The method of claim 1 wherein the as-cast article comprises an equiaxed region with an average grain size of  $289 \pm 42 \mu\text{m}$ .

16. A method of casting a creep-resistant Ni-based superalloy, the method comprising:

forming a feed stock comprising Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B); and

fabricating an as-cast article comprising creep-resistant Ni-based superalloy in a predetermined shape using the feed stock and at least one process comprising vacuum induction melting (VIM), electroslag remelting (ESR) and/or vacuum arc remelting (VAR), wherein fabricating the creep-resistant Ni-based superalloy comprises: melting the feed stock in a furnace, forming a liquid metal;

pouring the liquid metal into a preheated mold, forming a molten metal;

solidifying the molten metal in the preheated mold, forming the as-cast article; and

homogenizing the as-cast article, wherein homogenizing the as-cast article comprises a heating sequence of one hour at about 1075° C., three hours at about 1125° C., eight hours at about 1200° C. and eight hours at about 1250° C., wherein the homogenizing the as-cast article forms a specific element segregation below  $\pm 1\%$  variation from the nominal chemistry of these elements throughout the as-cast article.

17. The method of claim 16 wherein the as-cast article comprises an equiaxed region with an average grain size of  $289 \pm 42 \mu\text{m}$ .

18. A method of casting a creep-resistant Ni-based superalloy, the method comprising:

forming a feed stock comprising Nickel (Ni) and at least one of Chromium (Cr), Cobalt (Co), Aluminum (Al), Titanium (Ti), Niobium (Nb), Iron (Fe), Carbon (C), Manganese (Mn), Molybdenum (Mo), Silicon (Si), Copper (Cu), Phosphorus (P), Sulfur (S) and Boron (B); and

fabricating an as-cast article comprising creep-resistant Ni-based superalloy in a predetermined shape using the feed stock and at least one process comprising vacuum induction melting (VIM), electroslag remelting (ESR) and/or vacuum arc remelting (VAR), wherein fabricating the creep-resistant Ni-based superalloy comprises: melting the feed stock in a furnace, forming a liquid metal;

pouring the liquid metal into a preheated mold, forming a molten metal, wherein preheating the mold comprises heating the mold to about 300° C. to about 700° C. from about 10 minutes to about 5 hours;

solidifying the molten metal in the preheated mold, forming the as-cast article; and

homogenizing the as-cast article, at least two of the sequential steps of treating the cast alloy: 0.5 to 5 hours

at  $1075\pm25^\circ\text{ C.}$ ; 1.5 to 3 hours at  $1125\pm25^\circ\text{ C.}$ ; 3 to 15 hours at  $1200\pm25^\circ\text{ C.}$ ; 3 to 24 hours at  $1250\pm25^\circ\text{ C.}$ , wherein the homogenizing the as-cast article forms a specific element segregation below  $\pm1\%$  variation from the nominal chemistry of these elements throughout the as-cast article. 5

**19.** The method of claim **18** wherein the as-cast article comprises an equiaxed region with an average grain size of  $289\pm42\text{ }\mu\text{m.}$

\* \* \* \* \*

10